

Jan. 10, 1967

K. A. MACDONALD ETAL

3,297,901

DISPENSER CATHODE FOR USE IN HIGH POWER MAGNETRON DEVICES

Filed June 5, 1964



FIG. 1



FIG. 2

INVENTORS.  
KENNETH A. MACDONALD  
and JOSEPH A. SMITH

David M. Keay  
AGENT.

## 1

3,297,901

## DISPENSER CATHODE FOR USE IN HIGH POWER MAGNETRON DEVICES

Kenneth A. Macdonald and Joseph A. Smith, Williamsport, Pa., assignors, by mesne assignments, to Litton Industries, Inc., Beverly Hills, Calif., a corporation of Delaware

Filed June 5, 1964, Ser. No. 372,804

16 Claims. (Cl. 313—346)

This invention relates to emissive cathodes, particularly to indirectly heated electron emissive dispenser cathodes for use in high power magnetron devices.

Cathodes employed as the electron source in magnetron devices are commonly dispenser type cathodes in which an alkaline earth metal composition is dispersed throughout a matrix of a refractory metal. Cathodes of this type may be fabricated as by impregnating a porous tungsten body with an alkaline earth compound, or by compacting and sintering a mixture of an alkaline earth compound with one or more refractory metals. The alkaline earth composition chosen is normally one which will be slowly reduced by the refractory metal at the operating temperature of the cathode to provide free alkaline earth metal at the emissive surface of the cathode, thereby enhancing the electron emitting capabilities of the surface and producing a copious supply of primary electrons.

As is well known in the operation of pulsed magnetrons, electrons from the cathode which are not in proper phase to contribute energy to the oscillating mode of the magnetron return to the cathode. Since the returning electrons strike the cathode with considerable energy, secondary electrons are expelled and the cathode is heated. After oscillation has been started, the cathode heater current is reduced and the necessary energy for heating the cathode is largely obtained from the back bombardment by the electrons returning to the cathode. In high power magnetrons, secondary electrons are the principal constituent of the cathode current; therefore, dispenser type cathodes for use in high power magnetrons commonly employ materials which have good secondary emission capabilities in addition to their primary electron emission capabilities. A frequently used example of such a cathode is a porous tungsten body impregnated with barium calcium aluminate.

As mentioned above, the plentiful supply of primary electrons from a dispenser type cathode depends on the availability of an adequate quantity of free alkaline earth metal at the emissive surface of the cathode. However, the quantity of free alkaline earth metal produced by cathodes most commonly used in magnetrons is more than sufficient for this purpose, and some of the excess material evaporates from the surface of the cathode and deposits on adjacent elements of the magnetron structure, such as the cathode and shields, the magnet pole pieces, and the anode vane tips. The free alkaline earth metal causes spurious electron emission from these elements which interferes with the proper oscillating mode of the magnetron.

Various techniques have been employed in attempting to avoid the excessive production of free alkaline earth metal. For example, the conventional impregnated tungsten cathode may be operated at a lower temperature, or special cathodes may be fabricated employing materials which have good secondary emission capabilities but a low rate of evaporation of alkaline earth metal, and consequently low primary emission. However, high power magnetrons employing cathodes of these types frequently have poor starting stability. That is, the magnetron may not start to oscillate immediately upon the

## 2

application of the full pulsed voltage. The poor starting characteristics of these devices appear to be due to the fact that the cathode produces little or no free alkaline earth metal at the operating temperature, and therefore the cathode surface is susceptible to deactivation by poisoning.

It is an object of the present invention, therefore, to provide an improved cathode.

It is a more specific object of the invention to provide a dispenser type cathode which is capable of producing sufficient primary electrons to provide immediate starting of a high power magnetron but which does not evaporate an excessive quantity of emission enhancing material.

Briefly, in accordance with the foregoing objects, a cathode according to the invention comprises a major surface region of a material capable of emitting secondary electrons and a minor surface region of a material which provides a source of primary electrons. The minor surface region of the cathode may be constituted of a material which in itself is a good primary emitter of electrons or it may be of a reducing material which reduces non-emitting compounds diffusing from the major surface region to form a low work function material, thereby creating a region of high primary emission at the interface between the reducing material and the major surface region.

Additional objects, features, and advantages of cathodes according to the invention will be apparent from the following detailed discussion and the accompanying drawings wherein:

FIG. 1 is a cross-sectional view in elevation of a portion of a magnetron having mounted therein a cathode according to one embodiment of the invention, and

FIG. 2 is a cross-sectional view illustrating a cathode according to another embodiment of the invention.

A magnetron incorporating the first embodiment of the invention is illustrated in FIG. 1. The magnetron includes a cylindrical anode block 10 having a plurality of vanes 11 extending radially inward therefrom to provide a plurality of cavity resonators lying in a circular array about the central axis of the anode. The anode is strapped with pairs of concentric metal rings 12 located in recesses in each end of the vanes. Each strapping ring is connected only to alternate vanes in the manner well known in the art in order to insure operation of the magnetron in the  $\pi$  mode. Upper and lower magnet pole pieces 13 and 14 are sealed to the anode block and are arranged to direct a magnetic field from permanent magnets (not shown) through the magnetron interaction space. Electromagnetic energy is coupled from the device by an output coupler 15 communicating with one of the cavity resonators.

An electron emissive cathode 20 according to the invention is positioned centrally of the anode and spaced from the tips of the vanes. The cathode is brazed to a cathode support 21 and passes through a bore 22 in the lower pole piece 14. The cathode support 21, and pole piece 14 are attached together by a suitable arrangement of insulating hermetic seals (not shown).

The cathode 20 includes a hollow cylindrical sleeve 25 of molybdenum which is sealed at its lower end to the cathode support 21 and which extends centrally of the anode up into a recess 26 in the upper magnet pole piece. Non-emissive end shields 27 and 28 are staked to steps on the molybdenum sleeve so as to confine the electrons and prevent their movement into the end spaces above and below the ends of the anode vanes. The end shields are separated from the electron emissive surface 30 of the cathode by molybdenum spacers 31 and 32. A coiled heater element 33 of tungsten wound on a ceramic mandrel 34 is positioned centrally of the molybdenum sleeve

25. One end of the heater element is electrically connected to the cylindrical sleeve 25. The lower end of the heater element extends through a spacer 35 in the bottom of the sleeve and passes externally of the magnetron through a suitable arrangement (not shown) to provide a terminal for supplying heater current to the heater element.

In the cathode according to the invention as illustrated in FIG. 1 the active surface of the cathode includes a first or major surface region 40 having a material at the surface which is capable of emitting secondary electrons and has a low rate of evaporation of emission enhancing material. Adjoining the ends of this region are two minor surface regions 41 and 42, each of which provides a source of primary electrons. The area of the minor surface regions is small relative to the area of the major surface region.

The major surface region 40 is formed of a cylinder of material which is a good secondary emitter of electrons but which has a low rate of evaporation of free alkaline earth metal. The cylinder may be a matrix of refractory metal having dispersed therein a series of compounds of an alkaline earth metal of the nature of, for example, tungstates and molybdates which are not readily reduced to the free alkaline earth metal by the refractory metal.

More specifically, the cylinder may be formed by compacting a mixture of barium carbonate and one or more refractory metals such as tungsten and molybdenum and sintering at a high temperature in an inert atmosphere. Under such conditions tungstates and/or molybdates of barium are formed. Alternatively, the cylinder may be of porous tungsten, molybdenum, or rhenium impregnated with tungstates or molybdates of an alkaline earth metal such as barium.

The minor surface regions 41 and 42 are formed of cylinders coaxial with the cylinder forming the major surface region and adjoining each end of the major surface region. Each cylinder may be a matrix of refractory metal having dispersed therein an alkaline earth metal composition capable of furnishing alkaline earth metal to the surface of the cylinder. More specifically, the cylinders may be annular members or washers of porous tungsten impregnated with a barium calcium aluminate of relatively low barium content.

Alternatively, the minor surface regions 41 and 42 may be formed of a material which is of strongly reducing nature such that non-emitting compounds diffusing from the adjoining secondary emitting region are reduced and a low work function material is formed, thereby creating a region of high primary emission at the interface between the major and minor surface regions. More specifically, rings or washers of tantalum, zirconium, titanium, or niobium may be employed, tantalum being preferred.

The total surface area of the minor surface regions 41 and 42 desirably should be of the order of 20% or less of the total emission surface area of the cathode. Specifically, cathodes have been fabricated in which the major surface region 40 was provided by a cylinder .100 inch high of a compacted mixture of 10% by weight barium carbonate, 45% by weight tungsten, and 45% by weight molybdenum, sintered at 1700° C. in pure dry nitrogen. This cylinder was employed with two washers 41 and 42 each .010 inch thick of porous tungsten impregnated with barium calcium aluminate of the composition



Alternatively, tantalum washers .010 inch thick have been employed in place of the impregnated tungsten washers.

FIG. 2 illustrates a second embodiment of a cathode 50 according to the invention which may be mounted in the magnetron of FIG. 1. In this embodiment the cylindrical surface of secondary electron emitting material is provided by two cylinders 51 and 52. Intermediate the

5 two cylinders and adjoining an end of each is a narrow cylindrical region 53 of material providing a source of primary electrons. The materials employed for producing primary and secondary electron emission may be the same materials as those employed in the first embodiment of the invention.

Cathodes according to the invention have been utilized in high power magnetrons with excellent results. Starting stability has been satisfactory indicating that sufficient free alkaline earth metal is available at the surface of the minor surface regions to keep the surface active and not susceptible to deactivation by poisoning. Interference with the proper operating mode of the device has been eliminated indicating that there is no significant excess of free alkaline earth metal available to establish sources of spurious electrons on elements of the device adjacent the cathode.

What is claimed is:

1. A cathode comprising a first surface region of material capable of emitting secondary electrons and having a low rate of evaporation of emission enhancing material, and a second surface region of material providing a source of primary electrons.
2. A cathode comprising a first surface region of material having a high secondary electron emission yield and a low rate of evaporation of free alkaline earth metal, and a second surface region of a refractory metal having dispersed therein an alkaline earth compound capable of furnishing primary electron emission at the surface adjoining the first surface region, the surface area of the second surface region being small relative to the surface area of the first surface region.
3. A cathode according to claim 2 in which said first surface region comprises a matrix of refractory metal having dispersed therein compounds of an alkaline earth metal which are not readily reduced to free alkaline earth metal by the refractory metal of the matrix.
4. A cathode according to claim 2 in which said first surface region comprises a matrix of refractory metal selected from the group consisting of tungsten, molybdenum, and rhenium having dispersed therein a material selected from the group consisting of tungstates and molybdates of an alkaline earth metal.
5. A cathode according to claim 2 in which said first surface region comprises a material produced by compacting and sintering a mixture of an alkaline earth metal carbonate and a refractory metal selected from the group consisting of tungsten and molybdenum.
6. A cathode comprising a first surface region of material having a high secondary electron emission yield and a low rate of evaporation of free alkaline earth metal, and a second surface region of material capable of reducing non-emitting compounds diffusing from the first surface region to create a region of primary electron emission at the interface of the first and second surface regions, the surface area of the second surface region being small relative to the surface area of the first surface region.
7. A cathode according to claim 6 in which said first surface region comprises a matrix of refractory metal having dispersed therein compounds of an alkaline earth metal which are not readily reduced to free alkaline earth metal by the refractory metal of the matrix.
8. A cathode according to claim 6 in which said first surface region comprises a matrix of refractory metal selected from the group consisting of

tungsten, molybdenum, and rhenium having dispersed therein a material selected from the group consisting of tungstates and molybdates of an alkaline earth metal.

9. A cathode according to claim 6 in which said first surface region comprises a material produced by compacting and sintering a mixture of an alkaline earth metal carbonate and a refractory metal selected from the group consisting of tungsten and molybdenum. 5

10. A cathode according to claim 6 in which said second surface region comprises a refractory metal selected from the group consisting of tantalum, niobium, zirconium and titanium. 10

11. A cylindrical cathode comprising 15  
a first material comprising a matrix of refractory metal having dispersed therein compounds of an alkaline earth metal which are not readily reduced to the free alkaline earth metal by the refractory metal,  
a second material comprising a matrix of refractory 20 metal having dispersed therein an alkaline earth metal composition capable of furnishing primary electron emission at the surface,  
a first cylindrical body constituted of one of said materials,  
a second cylindrical body constituted of the other of 25 said materials coaxial with the first cylindrical body and adjoining the first cylindrical body at one end thereof, and  
a third cylindrical body constituted of the other of said materials coaxial with the first and second cylindrical bodies and adjoining the first cylindrical body at the other end thereof,  
the cylindrical surface area of the second material being less than 20% of the cylindrical surface area 30 of both the first and second materials.  
35

12. A cathode according to claim 11 in which said first material comprises a material produced by compacting and sintering a mixture including by weight about 10% barium carbonate, 45% tungsten, 40 and 45% molybdenum, and

said second material comprises a porous tungsten body impregnated with barium calcium aluminate of composition  $BaO \cdot 2CaO \cdot 2Al_2O_3$ .

13. A cathode according to claim 11 in which 45 said first material comprises a porous tungsten matrix impregnated with tungstates of barium,

said second material comprises a porous tungsten body impregnated with barium calcium aluminate of composition  $BaO \cdot 2CaO \cdot 2Al_2O_3$ .

14. A cylindrical cathode comprising  
a first material comprising a matrix of refractory metal having dispersed therein compounds of an alkaline earth metal which are not readily reduced to the free alkaline earth metal by the refractory metal,  
a second material capable of reducing non-emitting compounds diffusing from the first material to create a region of primary electron emission at interfaces between the first and second materials,  
a first cylindrical body constituted of one of said materials,  
a second cylindrical body constituted of the other of said materials coaxial with the first cylindrical body and adjoining the first cylindrical body at one end thereof, and,  
a third cylindrical body constituted of the other of said materials coaxial with the first and second cylindrical bodies and adjoining the first cylindrical body at the other end thereof,  
the cylindrical surface area of the second material being less than 20% of the cylindrical surface area of both the first and second materials.

15. A cathode according to claim 14 in which said first material comprises a material produced by compacting and sintering a mixture including by weight about 10% barium carbonate, 45% tungsten, and 45% molybdenum, and

said second material comprises a washer of tantalum.

16. A cathode according to claim 14 in which said first material comprises a porous tungsten matrix impregnated with tungstates of barium,  
said second material comprises a washer of tantalum.

#### References Cited by the Examiner

#### UNITED STATES PATENTS

- |           |         |                 |       |           |
|-----------|---------|-----------------|-------|-----------|
| 2,698,913 | 1/1955  | Espersen        | ----- | 313—346   |
| 2,957,100 | 10/1960 | Espersen et al. | ----- | 313—346   |
| 3,027,489 | 3/1962  | Tuinila et al.  | ----- | 313—346 X |

45 JOHN W. HUCKERT, *Primary Examiner.*

A. J. JAMES, *Assistant Examiner.*